

Aug. 10, 1926.

1,595,803

W. J. MERTEN

HELICAL SPRING QUENCHING DEVICE

Filed March 5, 1921



Fig 1



Fig 2.



Fig 3.

WITNESSES:

*John W. Whiting*  
*H.C. Biernan*

INVENTOR

*William J. Merten.*

BY

*Merle G. Clark*  
ATTORNEY

## UNITED STATES PATENT OFFICE.

WILLIAM J. MERTEN, OF PITTSBURGH, PENNSYLVANIA, ASSIGNOR TO WESTINGHOUSE ELECTRIC & MANUFACTURING COMPANY, A CORPORATION OF PENNSYLVANIA.

## HELICAL-SPRING-QUENCHING DEVICE.

Application filed March 5, 1921. Serial No. 449,637.

This invention relates to quenching, more especially to the quenching of hollow bodies, such as helical springs used in railway rolling stock.

Considerable difficulty has been encountered in quenching helical springs in order to harden the same. It has been found that, when springs of this character are heated to a temperature above the critical point of the material and the spring placed in a quenching bath, the hardness of the various parts of the spring is not uniform. Apparently, the quenching or cooling in the medium is not uniform throughout and, generally, the outer surfaces of the coils of the springs are harder than the inner surfaces. This is probably due to a difference in the rate of cooling of the surfaces that sets up strains in the spring which cause failure thereof.

The present invention is designed to obviate this difficulty, it being among the objects of this invention to quench hollow bodies, such as helical springs, in such manner as to avoid the non-uniformity of hardness which has hitherto resulted from quenching in liquid media and to provide a spring of this character in which substantially no strains are set up between the various parts thereof.

I have found that, when a hollow body, such as a helical spring, is heated to a high temperature and then dropped into a bath of quenching fluid, such as oil, there is less circulation of oil in the interior of the spring than along its outer surfaces. Gas pockets are formed in the interior which tend to reduce the circulation of oil in the interior of the spring and thus further retard the hardening process.

I have overcome these difficulties by providing a system in which the quenching fluid, such as oil, is forced simultaneously through the interior of the spring and over the outer surface thereof in order to cause uniform and simultaneous hardening of the entire spring. By providing such a system, I have formed springs of uniform hardness throughout and have greatly diminished the danger of breaking of such springs in service and have prolonged the life and efficiency thereof.

In practicing my invention, I provide a bath of quenching fluid, such as oil, and sus-

pend therein a suitably shaped member adapted to hold a spring to be quenched in a horizontal position. I further provide a conduit having a series of openings and place it above the spring to be quenched so that liquid flowing from said openings flows over the exterior of the spring. A second conduit is so placed that liquid flowing therefrom passes through the interior of the spring. Both conduits are connected to a source of pressure which forces the oil therethrough.

In the accompanying drawings forming a part hereof and which illustrate a single embodiment of my invention,

Fig. 1 is a vertical, sectional view through a container embodying my invention;

Fig. 2 is a side elevational view of the quenching means, and

Fig. 3 is a front view of the spring holder.

I provide a container 1, preferably open at the top and filled with quenching fluid 2 of any suitable kind, usually oil. A pipe 3, connected to a source of oil under pressure, leads into container 1 and has a branch or T 4 to which is connected a nipple 5 having a valve 6 connected thereto and terminating in a short pipe 7. To the other opening of the T 4 is secured a valve 9 having a pipe 8 connected thereto, said pipe terminating at 10 in a horizontal member, the end thereof being closed as shown at 11. Openings 12 are formed in the lower portion of horizontal section 10.

Directly below said portion 10 is placed a member 13 of scoop shape having a series of openings 14 and secured to a frame 15 having a bend 16 of substantially the form of an inverted U. A co-operating hook member 17 is suspended from a suitable support 18 secured to the container 1. A pipe 19 leads from the bottom of the container to the source of pressure and aids in the circulation of the oil.

The operation of my device is as follows: Oil is caused to flow into pipe 3 under pressure produced by a pump or other suitable means (not shown) and flows through the T 4 and valves 6 and 9 and out through pipes 7 and 8. The openings of the valves are regulated to give the desired flow. A spring 20 to be quenched is placed upon the member 13 and is lowered into the bath

of quenching fluid, being suspended there-  
in from hook member 17. Oil, flowing from  
openings 12, descends upon the exterior of  
the spring while oil flows from the open end  
5 of pipe 7, which is centrally located with  
respect to the interior of the spring, thus  
causing a rapid circulation of oil on all sides  
of the spring. Openings 14 in member 13  
serve to allow a free circulation of oil  
10 along the underside of the spring and, at  
the same time, the support of member 13  
prevents distortion of the spring which  
would take place if it were not properly  
held in position during the quenching opera-  
15 tion.

It will be apparent that my invention  
provides a novel method of quenching hollow  
bodies, such as spiral springs, in that  
both the exterior and the interior thereof  
20 are quenched simultaneously. When the oil  
is caused to flow under pressure, the quench-  
ing operation is expedited and the efficiency  
of the process is increased. By causing uniform  
25 quenching of the spring, it becomes  
of uniform hardness on all sides, and the  
danger of the spring breaking in service is  
minimized.

I have found that the direction of the  
two streams of the incoming cooling fluid  
30 at right angles to each other is important.  
The delivery of cooling fluid at a substan-  
tial pressure to the center of the spring and  
into the narrow spaces between the coils  
thereof avoids the formation of gas pockets  
35 therein and thereby accelerates the abstraction  
of heat from the spring being treated.  
Convection currents are induced around the  
spring, keeping the oil at a uniformly low  
temperature at and in the vicinity of the  
40 spring. This may be materially increased  
by having the horizontal pipe 10 at approxi-  
mately the level of the oil and the spring  
approximately six inches below the surface  
of the oil. This results in a spring which is  
45 hardened uniformly and greatly strength-  
ened by reason of the minimizing of strains  
induced in the spring by the hardening  
operation.

I claim as my invention:

50 1. A method of quenching a hollow body  
which comprises simultaneously directing  
streams of quenching fluid radially and  
axially on said body.

55 2. A method of quenching a helical spring  
which comprises causing quenching fluid

to flow into contact with both the interior  
and the exterior thereof.

3. A method of quenching a helical spring  
which comprises causing quenching fluid to  
flow into contact with both the interior and  
the exterior thereof simultaneously.

4. A method of quenching a helical spring  
which comprises supporting the same longi-  
tudinally and causing quenching fluid to  
flow into contact with both the interior and  
the exterior thereof.

5. A method of quenching a helical spring  
which comprises placing the same on a per-  
forated support and causing quenching  
fluid to flow into contact with both the in-  
terior and the exterior thereof.

6. Apparatus for quenching hollow bodies  
comprising a container for quenching fluid,  
a plurality of conduits for circulating said  
fluid and means for holding a body to be  
75 quenched in the path of currents so gener-  
ated, one of said conduits being positioned  
at the surface of said fluid.

7. Apparatus for quenching hollow bodies  
comprising a container for quenching fluid,  
a plurality of conduits connected to a com-  
mon source for circulating said fluid and  
means for holding a body to be quenched in  
80 the path of currents so generated, one of  
said conduits being horizontal and posi-  
tioned at the surface of said fluid.

8. Apparatus for quenching hollow bodies  
comprising a container for quenching fluid,  
a plurality of conduits for circulating said  
fluid and means for holding a body to be  
90 quenched in the path of currents so gener-  
ated, said means comprising a perforated  
member of scoop shape and means for sus-  
pending the same in said container.

9. Apparatus for quenching hollow bodies  
comprising a container for quenching fluid,  
a plurality of conduits for circulating said  
fluid, means for holding a body to be  
95 quenched in the path of currents so gener-  
ated, said means comprising a perforated  
member of scoop shape and means for sus-  
pending the same in said container, one of  
100 said conduits being adapted to circulate said  
fluid through said body and the other to  
force the same over said body.

In testimony whereof, I have hereunto  
subscribed my name this 26th day of Febrary  
1921.

WILLIAM J. MERTEN